

# UNITED STATES PATENT OFFICE.

JOHN M. RENO, OF KEWANNA, INDIANA.

## COMPOUND FOR USE WITH RAZOR-STROPS.

No. 879,319.

Specification of Letters Patent.

Patented Feb. 18, 1908.

Application filed September 20, 1907. Serial No. 393,812. (Specimens.)

To all whom it may concern:

Be it known that I, JOHN M. RENO, a citizen of the United States, residing at Kewanna, in the county of Fulton and State of Indiana, have invented certain new and useful Improvements in a Compound for Use with Razor - Strops, of which the following is a specification.

This invention relates to improvements in compounds for use with razor strops, and has for its objects, the provision of means whereby such articles may be rendered pliable and productive of the best attainable results; furthermore to maintain such strops in condition for immediate service and which will operate more effectively and expeditiously than those in common use. These objects are attained by the combination and treatment, in a certain manner, of such strops and a compound hereinafter fully described and claimed.

My compound consists of the following ingredients combined in the preparation stated, viz:

|    |            |      |
|----|------------|------|
| 25 | Iron oxid  | 10%  |
|    | Rouge      | 10%  |
|    | Crocus     | 10%  |
|    | Glycerin   | 5%   |
|    | Petrolatum | 15%  |
| 30 | Spermaceti | 5%   |
|    | Tallow     | 45%  |
|    |            | 100% |

These ingredients are to be thoroughly mingled by agitation, the same resulting in a reddish colored paste with the consistency of ordinary butter.

To the hook 1, is attached the link 2, connecting with the upper cross bar 3, of the strop 4, which is provided with a similar bar 5, at the lower end and connected with the handle 6.

In use, the operator grasps the handle, draws the strop towards him with enough force for the purpose required, and proceeds to manipulate the razor on the surface of the strop,—here shown as comprised of a fabric,

but which may be leather or other preferred material.

As such razor strops usually hang for long 50 continued periods, they naturally collect dust from the atmosphere and, even if pliable and in good condition originally, soon become dry and lose their usefulness, at least to an extent undesirable. 55

My invention consists in first cleansing the surface of the strop from dust and other accumulations by scraping, or even washing, if the surface be dry and hard.

The oxid of iron, rouge, and crocus give 60 the necessary cutting or abrasive qualities, the tallow and spermaceti afford a desirable body for holding the powder in the interstices of the material, the petrolatum softens and renders the strop pliable and the glycerin 65 prevents it from drying.

Only occasional treatment is necessary, depending on the temperature and quantity of dust atoms in the surrounding air.

I am aware that emollients and abrasives 70 have before been used for this purpose but am unadvised that a preparation of like properties has been employed.

Therefore, what I claim as new and desire to secure by Letters Patent is: 75

A compound for use with razor strops consisting of,

|            |      |
|------------|------|
| Iron oxid  | 10%  |
| Rouge      | 10%  |
| Crocus     | 10%  |
| Glycerin   | 5%   |
| Petrolatum | 15%  |
| Spermaceti | 5%   |
| Tallow     | 45%  |
|            | 100% |

In testimony whereof I have signed my name to this specification in the presence of two subscribing witnesses.

JOHN M. RENO.

Witnesses:

C. M. SNEPP,  
S. B. ROTH.